

Aug. 9, 1927.

1,638,369

F. SKAUPY

COLORED INCANDESCENT LAMP BULB

Filed April 7, 1925



Inventor:  
Franz Skaupy,

by *Alfred S. Juntz*,  
His Attorney.

Patented Aug. 9, 1927.

1,638,369

# UNITED STATES PATENT OFFICE.

FRANZ SKAUPY, OF BERLIN, GERMANY, ASSIGNOR TO GENERAL ELECTRIC COMPANY, A CORPORATION OF NEW YORK.

## COLORED INCANDESCENT-LAMP BULB.

Application filed April 7, 1925, Serial No. 21,389, and in Germany May 17, 1924.

Colored incandescent lamp bulbs have previously been produced by making the bulb of colored glass, or by providing a bulb of clear glass with a colored coating, either 5 of colored glass, such as is commonly used in the ceramic industry, or of colored varnish. Colored bulbs produced as just described allow the filament to show through more or less and they do not give a good 10 diffusion of light or a good color effect. To overcome these disadvantages it has been proposed to add to the glass which is to be subsequently applied to the bulb of clear 15 glass a clouding medium such as that used in making the opal glaze generally used in the ceramic industry. However, as colored glazes in thin layers allow a good deal of light to pass, a comparatively thick layer 20 of colored glaze must be used in order to obtain the desired results. The use of thick colored glazes containing a clouding medium is accompanied by great difficulties, because 25 the addition of the clouding medium raises the fusing temperature at which the glazes melt on the bulb, and consequently undesirable cracks and deformations of the bulb are frequently produced in the very thin 30 walls of the lamp bulb. In addition, the thick glazes, when covering only a part of the bulb, may give rise to undesirable shadows.

The object of the invention is to overcome these defects and in accordance with the invention the bulb is composed of a translucent glass, such as that commonly known as 35 opal, milk, or mat glass, and a colored glaze, such as that commonly used in the ceramic industry and consisting of a low melting lead borate glass having a melting point lower 40 than that of the bulb glass and containing a suitable pigment, applied to the translucent bulb to cover it, either partly or entirely. In a bulb made in this way the colored coating or glaze serves only to obtain the color 45 effect, while the uniform diffusion of the light is produced by the translucent bulb itself, which acts as a foundation for the coating or glazes. The colored coating, particularly a glaze, can therefore be applied in a 50 very thin layer, which very greatly reduces the danger of damage to the bulb while the glaze is being fused, particularly if transparent colored glazes are used, because such glazes, as is well known, are more easily feasible than the cloudy glazes, and, therefore,

can be burned into the bulb at a lower temperature. By the use of a translucent foundation the further advantage is obtained that when the bulb is only partly covered by a colored glaze the covering stands out much 60 more effectively by contrast with the bare white parts of the translucent bulb. Furthermore, where the glaze coating is applied to only parts of the bulb the appearance of the bulb is not affected, because the glaze on 65 account of its extreme thinness does not project appreciably from the bulb.

The invention is illustrated in one form in the accompanying drawing in which is shown an incandescent lamp bulb provided 70 in accordance with this invention with belts or bands of colored coating or glaze.

The bulb (a) consists of a translucent white glass, such as that commonly known as opal, milk, or mat glass, which is a white 75 translucent glass producing a uniform diffusion of light. On the translucent foundation provided by the bulb the bands or belts (b) preferably made of a colored glaze, are applied in the form of layers of very slight 80 thickness.

The glaze may be applied to the bulb (a) in any well known manner. For example, the glaze may be powdered, applied to the bulb, and then the powdered bulb heated to a temperature too low to deform the bulb but high enough so that the glaze fuses or is burned into the bulb. It is also possible before fusing or burning in the powdered glaze, to mix it with water, or if desired with 85 alcohol, and thereby produce a paste which may be applied to the bulb by a brush or a squirting device. The methods above described are particularly useful where the bulb is to be provided with belts or bands of 90 colored glaze. Where the entire bulb is to be covered with a uniform layer, the glaze may be applied in any of the ways above described or the bulb may be dipped bodily 95 into the paste made of powdered glaze mixed with water or alcohol.

These bulbs are useful for not only incandescent lamps, but any other lamps having a light source of high intrinsic brilliancy, such as an arc lamp, and may also be used to advantage for lamps in which the light is produced by a discharge through gas.

What I claim as new and desire to secure by Letters Patent of the United States, is:—

1. A lamp bulb of translucent glass hav-

ing on a part of its surface a thin adherent coating of glaze having a melting point lower than that of said glass and differing in color from the bulb.

5 2. A lamp bulb of white translucent glass having on it a thin adherent coating of a vitreous glaze of lower melting point and different color than said glass.

3. A lamp bulb of white translucent glass having on it a band of thin vitreous glaze of <sup>10</sup> lower melting point and different color than said translucent glass.

In witness whereof, I have hereunto set my hand this 19th day of March, 1925.

FRANZ SKAUPY.